

United States Patent [19]  
Bieber

[11] 3,837,847  
[45] Sept. 24, 1974

[54] CORROSION RESISTANT FERRITIC  
STAINLESS STEEL

[75] Inventor: Clarence George Bieber, West  
Milford, N.J.

[73] Assignee: The International Nickel Company,  
Inc., New York, N.Y.

[22] Filed: Dec. 23, 1971

[21] Appl. No.: 211,740

Related U.S. Application Data

[63] Continuation-in-part of Ser. No. 841,138, July 11,  
1969, abandoned.

[52] U.S. Cl. 75/128 W, 75/124, 75/128 T,  
75/128 G

[51] Int. Cl. C22c 39/20, C22c 37/10

[58] Field of Search 75/128 W, 126 C, 124

[56] References Cited

UNITED STATES PATENTS

2,051,415 8/1936 Payson ..... 75/128 W

|           |         |                  |          |
|-----------|---------|------------------|----------|
| 2,083,524 | 6/1937  | Payson .....     | 75/128 W |
| 2,110,891 | 3/1938  | Reitz .....      | 75/126 C |
| 2,141,016 | 12/1938 | Payson .....     | 75/128 W |
| 2,183,715 | 12/1939 | Franks .....     | 75/126 C |
| 2,518,715 | 8/1950  | Payson .....     | 75/126   |
| 2,624,671 | 1/1953  | Binder .....     | 75/126 C |
| 3,152,934 | 1/1964  | Lula .....       | 75/128 W |
| 3,177,577 | 4/1965  | Fujimura .....   | 75/128 T |
| 3,567,434 | 3/1971  | Richardson ..... | 75/128 W |

Primary Examiner—Hyland Bizot

Attorney, Agent, or Firm—Ewan C. MacQueen;  
Raymond J. Kenny

[57]

ABSTRACT

A ferritic stainless steel resistant to pitting and crevice corrosion and containing in addition to iron, correlated amounts of chromium, molybdenum, silicon, nickel and metal from the group consisting of titanium, vanadium and columbium. Other constituents can also be present.

13 Claims, No Drawings

## CORROSION RESISTANT FERRITIC STAINLESS STEEL

This application is a continuation-in-part of application Ser. No. 841,138 filed July 11, 1969 now abandoned.

As the metallurgist is aware, stainless steels since their inception have had a tremendous impact in virtually all segments of commercial and industrial activity. From small pins to huge vessels, from the most delicate of medical instruments to the most elaborate of chemical equipment, from food and dairy utensils to articles for handling the most acrid of acids and fumes, etc., these steels have played a significant role. And, in terms of the more exotic applications extensive research efforts are being pursued in such fields as aerospace and marine technology, including desalination, oceanography, etc.

Perhaps the principal reason for such diverse utility stems from the ability of stainless steels to resist the destructive influence of various corrosive media. Much has been written in explanation of the possible mechanisms involved, and it appears generally accepted that their corrosion resistant qualities are attributable, at least in part, to the ability to assume the "passive" condition. This is an inherent phenomenon due, it is believed, primarily to composition, mainly chromium, and involves the self-formation of a thin, continuous surface film (mostly chromium oxides) which acts as a protective barrier.

To be sure, all stainless steels do not resist all corrosive environments. One such steel might offer appreciable resistance to acid "X" but be quite susceptible to acid "Y," the opposite being true of a different stainless. And as is so often the case in which practically all members of a class of materials exhibit early or premature failure under a given circumstance, stainless steels in general have proven not to be an exception in certain chloride environments, e.g., "stagnant or slowly flowing" seawater.

By way of explanation and at the risk of oversimplification, there are any number of different types of corrosion, including general, pitting and crevice, intergranular, stress-corrosion cracking, etc.; however, it is the pitting and crevice form which is of greatest concern herein. As detailed in "The Corrosion Handbook" (1948) by Uhlig and in a number of other reference works, chloride ions (there are others) seem to display a peculiarly destructive talent in respect of the "passive condition" referred to above. This destructive manifestation normally occurs at "localized" surface areas which, for the lack of a better term, are simply referred to as "flaws" or "imperfections" (in operation they serve as natural crevices, hence "crevice corrosion").

Needless to say, such flaws are, as a practical matter, impossible to avoid. They may take the form of surface dents, notches, nicks, scratches and the like, defects unintentionally induced. Or they may be inescapably brought about because of the form or shape of a particular article of manufacture — stranded cable, cable terminal sockets and valve seats being illustrative. Then, there are the historically troublesome crevices formed by the workings of nature as exemplified by the adherence of barnacles and other marine organisms, etc.

The corrosion breakdown that follows apparently involves the formation of an electrolytic cell in which the "localized" spot ostensibly serves as a point of concen-

tration for attack by chloride ions whereby an active anode is established, the cathode being a large passive area. The disparity in anode versus cathode area results in a considerable difference in potential which causes a significant flow of current with, as Uhlig puts it, "attendant rapid corrosion at the small anode."

When stainless steels are immersed in a chloride environment such as "stagnant or slowly flowing" seawater, a not inconsiderable number of them seem particularly vulnerable to crevice corrosion. The protective passive film is deemed, as mentioned above, to be primarily chromium oxide(s), meaning oxygen contributes to the passive condition. Upon rupture of the film if the velocity of seawater in a given case is significant, above say, 3 feet per second (fps), there is a replenishment of oxygen to the ruptured local site such that there is a tendency for the punctured surface to self heal by way of forming new chromium oxide. (Also, "rapidly" flowing seawater tends to prevent the adherence of barnacles and other organisms). In stagnant seawater, however, such is not always the case due to lack of available oxygen. Moreover, *inter alia*, the acidity of soluble corrosion products, e.g., ferrous chloride, inhibits restoration of "passivity."

It has now been discovered that stainless steels containing chromium, molybdenum and nickel and other constituents as described herein offer greatly improved resistance to the destructive effects of chlorides, provided the constituents are properly correlated in terms of chemistry and provided further they are at least substantially if not completely ferritic in microstructure. Furthermore, the ferritic structure notwithstanding, steels in accordance herewith also manifest good notch toughness qualities, various compositions displaying satisfactory brittle-to-ductile notch toughness even down to temperatures as low as or lower than zero °F.

The foregoing combination of characteristics can be contrasted with at least certain of the literature. The Metals Handbook, for example, 8th ed., 1961, pages 554, 558-564, indicates that stainless steels perform well in seawater in the absence of fouling mechanisms (crevices) and if the velocity is 5 fps or greater. Similarly, in Stainless and Heat-Resisting Steels, L. Colombe and J. Hochmann, 2d. ed., (1965), p. 51, the ferritic 16-18 percent chromium grades are said to "... offer good seawater corrosion resistance provided the water is *not* stagnant and marine organisms are absent." And as to the known 25-30 percent chromium ferritic stainless steels the authors report them (p. 55) as being objectionable by reason of:

"Thus, a steel with 25% chromium melted under normal commercial conditions will give low impact values even at carbon contents as low as 0.03%, after heat treatment at any temperature between 800°C. and 1,200°C. and whatever the cooling conditions. This is a most troublesome fact and a major obstacle to the large scale industrial development of the steels. The difficulty is in fact notch sensitivity and nothing else; . . . ."

In addition to corrosion resistance and toughness, steels in accordance herewith also manifest good tensile strength and tensile ductility, yield strengths as high as 125,000 psi and ultimate tensile strengths upwards of 160,000 - 170,000 psi being attainable upon age hardening.

In any case, it is an object of the present invention to provide stainless steels novel in composition and which afford improved resistance to the corrosive effect of various chloride environments.

It is a further object to provide stainless steels having a ferritic or substantially ferritic microstructure and which exhibit satisfactory notch toughness characteristics.

Generally speaking, the present invention contemplates, subject to the qualifications described herein, stainless steels containing (by weight) from 16 to 30 percent, e.g., 18 to 22 percent chromium; from 0.5 up to about 11 percent, e.g., 3 to 11 percent, molybdenum; up to 3 percent, e.g., about 0.1 to 1.75 percent, silicon, the sum of the chromium plus three times the amount of molybdenum plus three times the percentage of silicon (referred to herein as the "CMS" indicator) being at least about 38 percent; from 2 percent, most advantageously, at least about 3 percent, and up to 8 percent nickel; up to less than 2 percent titanium; up to about 2 percent vanadium; up to about 2 percent columbium; up to 2 percent aluminum; up to 2 percent manganese; and the balance essentially iron.

In carrying the invention into practice, the chromium, molybdenum and any silicon must be correlated if satisfactory hot workability is to be achieved in addition to outstanding corrosion resistance. An alloy containing 20 percent chromium, for example, but molybdenum-free has been found to exhibit inferior corrosion resistance. On the other hand, an alloy containing, say, upwards of 30 percent chromium together with a molybdenum content of 10 percent is at best extremely difficultly, if at all, workable. Thus, where hot workability is a prerequisite the "CMS" factor should be less than 48 percent and beneficially not more than about 45 percent. Too, while silicon confers resistance to corrosion, it has been found to lessen ductility if present in excess of, say, 1.5 percent or 2 percent. For castings this qualification as to silicon need not obtain and in such instances (or in respect of other applications in which optimum ductility is not of necessity, e.g., deposit of an overlay on a substrate surface) the silicon content can be as high as 3 percent. No significant benefit is derived from higher silicon contents. For applications where it is important to minimize susceptibility to sigma formation, e.g., heavy sections, it is beneficial that silicon not exceed 0.5 or 0.75 percent.

Nickel portrays a most influential role by importantly contributing to high impact strength and low brittle-to-ductile transition temperatures. Charpy-V notch impact strengths of 15 foot-pounds or greater (a rather often used standard measurement) have been attained at temperatures well below -100°F. It is thought that such a characteristic would tend to mitigate the toughness drawback hitherto characteristic of high chromium ferritic steels. Nickel adds strength to the steels but must, however, be controlled for if present to the excess various characteristics including workability are impaired. A nickel range of from 3 or 4 percent to about 6 or 7 percent is deemed quite satisfactory.

While either air or vacuum melting techniques can be used in the preparation of the subject steels, at least one element from the group consisting of titanium, vanadium and columbium, particularly titanium, should be present in using air melting processing when the "CMS" indicator is not more than about 38 percent; otherwise, corrosion resistance suffers as will be illus-

trated herein. It has been found that a small but effective amount of one or more of these elements can markedly enhance corrosion resistance in various chloride media, e.g., ferric chloride. Should the "CMS" indicator be appreciably above 38 percent, e.g., 41 or 42 percent or more, air melting can be used in the absence of such constituents, but even under such circumstances (or notwithstanding the utilization of vacuum melting processing), one or more of these elements should be utilized, especially when the most drastic corrosion conditions are expected to be encountered. Furthermore, and apart from good corrosion resistance, in attaining good workability, e.g., forgeability and cold rollability, it is decidedly advantageous that at least titanium be present. The total sum of these constituents should not exceed about 4 percent and a range of about 0.15 percent or 0.2 to about 0.5 percent for each is satisfactory.

Aluminum can be used as a deoxidant but it does tend to impart a dross on the surface of air melted alloys in the molten condition and this can result in ingots with scabby surfaces. It can be present up to 2 percent, e.g., up to 1 percent since it seemingly promotes the effectiveness of the titanium, vanadium and columbium under air melting practice; but it need not exceed 0.1 or 0.2 percent. Actually, it is to advantage to use silicon to lieu of or together with a small amount of aluminum not only for its power in imparting good corrosion resistant qualities but also for deoxidation purposes as well.

As above set forth, it is important that the subject steels be characterized by a ferritic microstructure. Duplex structures such as those comprised of ferrite and a significant amount of austenite are to be avoided since corrosion resistance can be impaired. While a small or incidental amount of, say, austenite can be tolerated, e.g., up to 2, 3 or possibly 5 percent, the approach should be to avoid it. The same applies to phases other than austenite.

In the preparation of the instant steels the use of the purest materials commensurate with reasonable cost, (e.g., ferromolybdenum, ferrochromium and ingot iron) should be employed. Materials of exceptionally high purity, of course, can be utilized, e.g., molybdenum metal pellets, the electrolytic forms of iron, chromium and nickel, etc. As indicated above, both air melting and vacuum processing can be employed. Vacuum melting is, however, preferred since it has been found to promote higher notch-toughness characteristics (both resistance to impact and lower brittle-to-ductile impact transition temperatures), particularly in respect of columbium-containing steels. In addition to such techniques, other production practices are contemplated, including electroslag remelting, continuous casting and powder metallurgical processes.

A suitable pouring temperature is from about 2,800° to 2,900°F. As is commonly done in commercial steel-making practice for wrought products, ingots are preferably stripped hot from the mold and directly transferred to a soaking pit and soaked at a temperature of over 2,100° to 2,300°F. for a sufficient period and thereupon worked as by forging, hot rolling, etc. The hot finishing temperature can be as low as 1,400° to 1,500°F.

Following hot working, the steels can be annealed at a temperature of 1,900° to 2,100°F. prior to cold rolling. Surface defects are removed (e.g., by grinding, pol-

ishing) at appropriate intermediate stages but subsequent to final working. A final annealing treatment over the temperature range of 1,900° to 2,100°F. or 2,200°F. can be used; however, it is much preferred to use a temperature of 1,950° to 2,050°F., e.g., 2,000°F., 5 since the lower temperature would not only be more amenable to commercial practice but it is considered that corrosion resistance is likely to be superior. Holding periods at the lower annealing temperatures need not exceed about 10 to 15 minutes.

In order to give those skilled in the art a better appreciation of the invention, the following illustrative data are given.

A substantial number of alloys within the invention, Alloys 1 through 14, Table I, nominal compositions being given were prepared using air or vacuum melt processing. (AISI 316 and Alloys A through E are included in Table I for purposes of general comparison). An argon cover was used in the vacuum melt processing before adding the deoxidant calcium-silicon. This reduced the vacuum from about 29 in. Hg. to about 7 in. Hg. As to the air melted steels, a small amount of argon was continuously passed through the furnace but the amount was insufficient to completely prevent oxidation from taking place.

Ingots were soaked at about 2,200°F. to 2,300°F. and for the most part thereafter hot rolled to squares (either 2 × 2 inches or 1½ × 1½ inches or 1 × 1 inch). The specimens were then cut into two sections one of which was retained for stock purposes the other being rolled to ½ inch square bar. A portion of the ½ inch bar was removed for other testing, a part of the remainder being hot worked to about one-fourth inch thick, ground finished, annealed at 1,900° to 2,200°F., cold rolled to about 0.050 inch thick strip and final annealed at 2,000° or 2,100°F. Certain of the steels (4-6) were

reheated to 2,200° to 2,300°F. before rolling to ½ inch bar, steels A, B, D and 7 being reheated to 1,800°F. Steels C, 3, 7, 9-11 and 13 were additionally reheated to 2,100° or 2,150°F. prior to cold rolling.

Corrosion tests were conducted using an aggressive corrodent commonly used for test purposes, to wit, an aqueous 10 percent ferric chloride solution (Fe Cl<sub>3</sub>). The test specimens, having a surface area of approximately 25 square centimeters, were immersed for about 72 hours in the 10 percent ferric chloride solution, the temperature being maintained at about room temperature (approximately 72°F.); however, prior to immersion an intentional crevice was created about the surface of the specimens by wrapping a rubber band thereabout. This test being of an accelerated nature is deemed equivalent to an extreme long-time exposure in seawater and is described by M. A. Streicher in the Journal of the Electrochemical Society, Vol. 103, pp. 375-390, No. 7, July 1956.

The data in Table I reflect the excellent corrosion characteristics typical of alloys within the invention. This is in marked contrast to Alloys A through E and Alloy AISI 316. In comparision with steels in accordance herewith, AISI 316 failed catastrophically, undergoing near virtual disintegration. Note might be taken of Alloy E from which it may be observed that a nickel content of 10 percent seemed to adversely affect workability. Thus, it is beneficial that the nickel content not exceed 6 or 7 percent, a range of 2.5 to about 6 percent being quite suitable.

With further regard to Table I, Alloys A-D are indicative of what might be expected with low "CMS" values. As referred to herein, the "CMS" indicator should be at least about 38 percent. Even then, in consistently achieving outstanding resistance to pitting and crevice corrosion, particularly in the more drastic corrosive en-

TABLE I

| Alloy    | Cr | Ni   | Mo   | Ti   | Al   | Other              | Corrosion Behavior,<br>10% Fe Cl <sub>3</sub> |                   |
|----------|----|------|------|------|------|--------------------|-----------------------------------------------|-------------------|
|          |    |      |      |      |      |                    | Crevice<br>Corrosion                          | Wt. Loss,<br>Mgs. |
| AISI 316 | 17 | 12   | 2.5  | —    | —    | —                  | Very Heavy                                    | 2,592             |
| A        | 20 | n.a. | n.a. | 0.5  | 0.5  | 0.15 Si-Mn         | Very Heavy                                    | 3,610             |
| B        | 20 | 10   | n.a. | 0.5  | 0.5  | —                  | Very Heavy                                    | 7,910             |
| C        | 14 | n.a. | n.a. | n.a. | 0.5  | 0.15 Si-Mn, 0.12 C | Heavy                                         | 9,000             |
| D        | 26 | n.a. | n.a. | 0.5  | 0.5  | 0.15 Si-Mn         | Very Heavy                                    | 316               |
| E        | 20 | 10   | 8    | 0.5  | 0.25 | —                  | Broke On Forging                              | —                 |
| 1        | 18 | 2    | 8    | 0.5  | 0.5  | 0.15 Si-Mn         | None                                          | None              |
| 2        | 20 | 5    | 6    | 0.5  | 0.5  | —                  | None                                          | 0.5               |
| 3        | 20 | 6    | 6    | 0.5  | 0.25 | 0.25 Si            | Trace                                         | None              |
| 4        | 20 | 6    | 6    | 0.5  | n.a. | 0.35 Si            | Trace                                         | 0.4               |
| 5        | 20 | 6    | 6    | 0.25 | n.a. | 0.35 Si, 0.25 Cb   | None                                          | 0.1               |
| 6        | 20 | 6    | 6    | 0.25 | n.a. | 0.35 Si, 0.25 V    | None                                          | 0.6               |
| 7        | 20 | 4    | 8    | 0.5  | 0.5  | 0.15 Si-Mn         | None                                          | 0.6               |
| 8        | 20 | 4    | 8    | 0.4  | 0.25 | —                  | None                                          | 0.6               |
| 9        | 20 | 4    | 8    | 0.5  | 0.5  | —                  | None                                          | 0.6               |
| 10       | 24 | 2    | 5    | 0.5  | 0.5  | —                  | Very Slight                                   | 1.4               |
| 11       | 24 | 4    | 5    | 0.5  | 0.25 | —                  | None                                          | 0.7               |
| 12       | 26 | 5    | 4    | 0.5  | n.a. | 0.25 Si            | None                                          | None              |
| 13       | 28 | 4    | 3    | 0.5  | n.a. | 0.5 Si             | none                                          | None              |
| 14       | 28 | 5    | 4    | 0.5  | n.a. | 0.25 Si            | None                                          | None              |

n.a. = not added

\*Each alloy melt deoxidized with 0.05% calcium in the form of a 30% Ca - 70% Si master alloy.  
Balance of each composition was iron plus impurities.

vironments, it is of benefit that the "CMS" value be 39 percent or more; however, it is contemplated that where a high level of corrosion resistance is not consistently required, the "CMS" indicator can be as low as 35 or even down to 34 percent. Stainless steels having "CMS" indicators of 38 or 39 percent or more and compositions falling within the following ranges are deemed quite satisfactory: about 18 to 22 percent chromium, from about 5 to 10 percent molybdenum, up to about 2 percent silicon, from about 2.5 to 6 percent nickel, a small but effective amount of at least one constituent from the group consisting of up to 1 percent titanium, up to 1 percent vanadium and up to 1 percent columbium, up to about 1 percent aluminum and the balance essentially iron. Another highly suitable steel contains 22 to 28 percent chromium and 3.5 to 8 percent molybdenum, the remainder of the steel being the same as immediately above.

Steels in accordance herewith have also performed well corrosion-wise in media other than chlorides. Using the same general procedure described in connection with Table I, Alloy 7 was tested in 10 percent  $HNO_3$  and also in a solution containing 5 percent  $HNO_3$ , 5 percent  $H_2SO_4$  and 5 percent  $HCl$ . In the 10 percent  $HNO_3$  solution, a weight loss of but 0.1 milligram was experienced, the weight loss being slightly more, to wit, 0.7 milligram, in the multi-component solution. No crevice corrosion was detected. It might be added that the magnitude of corrosion resistance afforded by steels within the invention has been such as to render pickling of the steels exceedingly difficult in the annealed condition, e.g., when annealed at 1,950° or 2,000°F. or above. Thus, it is to be understood that the alloys of the subject invention can be used in many other corrosive environments apart from chlorides.

To demonstrate the effect of a constituent from the group consisting of titanium, vanadium and columbium on steels prepared by air melting practice, there is reported in Table II the corrosion resistant results obtained in respect of alloys both devoid of and containing titanium. These alloys (including vacuum melted alloys 17 and 18) were prepared and tested in generally the same manner as described in connection with Table I.

TABLE II

| Composition |    |    |    |      |      |                  | Corrosion Behavior,<br>10% $FeCl_3$ |           |
|-------------|----|----|----|------|------|------------------|-------------------------------------|-----------|
| Alloy       | Cr | Ni | Mo | Al   | Ti   | Other            | Crevice                             | Wt. Loss, |
|             |    |    |    |      |      |                  | Corrosion                           | mgs.      |
| F           | 20 | 2  | 8  | n.a. | n.a. | 0.15 Si, 0.25 Mn | Very Heavy                          | 418       |
| G           | 24 | 2  | 6  | n.a. | n.a. | 0.15 Si-Mn       | Very heavy                          | 8,320     |
| 15          | 20 | 2  | 8  | 0.5  | 0.5  | 0.15 Si, 0.25 Mn | None                                | 0.1       |
| 16          | 24 | 2  | 6  | 0.5  | 0.5  | 0.15 Si-Mn       | None                                | 1.9       |
| 17          | 20 | 4  | 8  | 0.25 | n.a. | —                | None                                | 0.6       |
| 18          | 20 | 4  | 8  | 0.25 | 0.4  | —                | None                                | 0.6       |
| 19          | 20 | 3  | 10 | 0.5  | 0.5  | 0.15 Si-Mn       | None                                | 1.8       |

n.a. = none added

0.05% Ca added in form of 30% Ca - 70% Si master alloy

Balance of composition iron and impurities

Alloys F and G are illustrative of the adverse effects to be expected using air melting processing without an element from the group titanium, vanadium and columbium. As demonstrated by Alloy 19, when the "CMS" indicator is appreciably above 38 percent (in this case nominally 40 percent) excellent corrosion resistant characteristics are obtainable using air melting techniques in the absence of each of the elements titanium, vanadium and columbium. However, Alloy 17 of Table II, a vacuum melted alloy, exhibited excellent corrosion resistance in ferric chloride maintained at room temperature. In conducting the same test but only using ferric chloride held at a temperature of approximately 122°F., this alloy manifested a loss of 549 milligrams and was noted by heavy crevice corrosion. A similar alloy, to wit, vacuum melted Alloy 18, but which nominally contained 0.4 percent titanium, showed only a loss of 0.4 milligram and very slight crevice corrosion when tested under the same conditions. Thus, as previously indicated, it is quite advantageous that one of these constituents be present.

Notch toughness characteristics are set forth in Table III concerning a series of alloys within (Alloys 20-26) and without (Alloy H) the invention. All were vacuum melted and oil quenched after annealing, Alloys 20-23, being annealed at 2,100°F., the others at 2,000°F. Liquid quenching has been found to offer better notch toughness, generally speaking, than say, air cooling. The combination of vacuum melting plus liquid quenching has been determined as consistently providing superior results as opposed to air melting or air cooling. It will be noted that excellent impact resistance and brittle-to-ductile transition temperatures (B.D.T.T.) are obtained particularly with alloys containing above 2 percent nickel, e.g., 4 to 6 percent nickel. (The brittle-to-ductile transition temperature (B.D.T.T.) is the temperature at which the steel specimen exhibited a minimum Charpy-V notch impact resistance of 15 foot-pounds). For a high chromium ferritic stainless steel, particularly one of exceptional corrosion resistant characteristics, to absorb an impact energy of over 100 foot-pounds or more at room temperature and to afford a transition temperature of minus 100°F. or lower, is quite unusual.

TABLE III

| Alloy No. | Cr | Ni | Mo | Al   | Ti  | Others     | C.V.N.,<br>ft.-lbs.<br>R.T. | B.D.T.T.<br>°F. |
|-----------|----|----|----|------|-----|------------|-----------------------------|-----------------|
| H         | 20 | 0  | 6  | n.a. | 0.5 | 0.5 Si     | 9                           | +200            |
| 20        | 20 | 2  | 8  | 0.5  | 0.5 | 0.15 Si-Mn | 24                          | —               |
| 21        | 20 | 4  | 8  | 0.5  | 0.5 | 0.15 Si-Mn | 92                          | -20             |
| 22        | 20 | 6  | 8  | 0.5  | 0.5 | 0.15 Si-Mn | 144                         | -130            |
| 23        | 20 | 8  | 8  | 0.5  | 0.5 | 0.15 Si-Mn | 124                         | -215            |
| 24        | 24 | 5  | 4  | n.a. | 0.5 | 0.25 Si    | —                           | -100            |
| 25        | 24 | 6  | 4  | 0.15 | 0.5 | —          | 151.5                       | -180            |
| 26        | 26 | 5  | 4  | n.a. | 0.5 | 0.25 Si    | —                           | -140            |

n.a. = not added

In Table IV representative data concerning tensile properties of steels within the invention are given. Yield strengths well above 100,000 psi are obtainable, particularly with steels containing more than 2 percent nickel, upon aging over a temperature range of above 800° to 1,000°F., e.g., 900°F., for a period of about 1 to 4 hours. The data is in respect of alloys in both the annealed (2,000° or 2,100°F.) and aged conditions (4 hours at 900°F.).

sistent with good commercial steel making practice. It is, at best, most difficult to avoid the presence of carbon and to do so could add to the cost. Carbon can remove undesirable oxygen but is not essential. It is advantageous that it be kept to low levels, e.g., below 0.02 to 0.04 percent. It can be tolerated in higher amounts up to 0.1 percent but above about 0.06 or 0.07 percent, it should be fixed. It is preferred that the carbon be fixed above about 0.02 percent. Nitrogen can be pres-

TABLE IV

| Alloy | Cr<br>% | Ni<br>% | Mo<br>% | Al<br>% | Ti<br>% | Y.S.<br>ksi | Annealed<br>U.T.S.<br>ksi | El.<br>% | Aged<br>Y.S.,<br>ksi | Aged<br>U.T.S.<br>ksi | El.,<br>% |
|-------|---------|---------|---------|---------|---------|-------------|---------------------------|----------|----------------------|-----------------------|-----------|
| 7     | 20      | 4       | 8       | 0.5     | 0.5     | 86.4        | 109.3                     | 24       | 116.9                | 152.0                 | 20        |
| 28    | 20      | 6       | 8       | 0.5     | 0.5     | 90.3        | 116.1                     | 25       | 127.3                | 174.1                 | 18        |
| 29    | 20      | 2       | 8       | 0.5     | 0.5     | 71.6        | 100.6                     | 28       | 83.1                 | 109                   | 26        |
| 30    | 20      | 8       | 8       | 0.5     | 0.5     | 80.3        | 110                       | 33       | 131                  | 153.4                 | 25        |
| 31    | 24      | 2       | 6       | 0.5     | 0.5     | 73.9        | 90.6                      | 30       | 81                   | 99                    | 31        |

Each alloy deoxidized with Ca-Si and Si-Mn.  
Balance of composition iron and impurities

A further attribute of the instant steels is that they possess a satisfactory fatigue life. Since it is not uncommon in assessing fatigue behavior to use a maximum fibre stress of at least equal to one-half of the tensile strength to ascertain whether a steel will perform adequately for a period of at least one hundred million cycles in duration, a smooth bar specimen of an alloy nominally containing 20 percent chromium, 6 percent nickel, 6 percent molybdenum, 0.5 percent silicon, 0.5 percent titanium, 0.15 percent calcium silicon, balance iron and impurities, was subjected to a maximum fibre stress of 58,000 psi. (The ultimate tensile strength upon annealing at 2,000°F. was 105,000 psi.) Using an R. R. Moore Rotating Beam Machine it was found that the specimen exhibited a life of over 114,000,000 cycles at which point the tested was discontinued.

Alloys within the invention are contemplated for general use in marine environments including seawater and sea atmospheres and in connection with such operations as off-shore drilling, desalination, undersea mining, etc. More specifically, they are considered useful for pumps and parts thereof (including vanes and impellers), propellers, pipe, valves, fasteners, tubing in general including tubing for both heat exchangers and desalination equipment, tube sheets, water boxes, seawater evaporators, shafting, sheathing, marine hardware, e.g., chocks, cleats, pulleys, oil well equipment, etc., components for paper pulp equipment and chemical plant equipment for the handling of oxidizing acids and salts thereof, containers for pressure vessels for the storage and transportation of various corrosive chemicals, etc. The steels can be produced in conventional mill forms including sheet, bar, plate, rod, etc., and also as castings.

As will be understood by those skilled in the art, the term "balance" or "balance essentially" when used in referring to the iron content does not exclude the presence of other elements commonly present as incidental elements, e.g., deoxidizing and cleansing elements, and impurities ordinarily associated therewith in small amounts which do not adversely affect the basic characteristics of the alloy. Elements such as sulfur, hydrogen and oxygen should be maintained at low levels con-

25 ent in usual amounts. Other constituents can be present as supplementary elements such as up to 4 percent tungsten and up to 10 percent cobalt. Tantalum is often found associated with columbium; however, it is heavy and costly as well as non-essential and should be held 30 to not above 0.2 percent.

Although the present invention has been described in conjunction with preferred embodiments, it is to be understood that modifications and variations may be resorted to without departing from the spirit and scope of 35 the invention, as those skilled in the art will readily understand. In this regard, zirconium can be used to replace titanium, vanadium or columbium in whole or in part but it is more beneficial for various reasons to use one or more of the latter. Such modifications and variations are considered to be within the purview and scope 40 of the invention and appended claims.

I claim:

1. A stainless steel having a substantially ferritic microstructure in the ferritic condition and possessing excellent resistance to the corrosive effects of such environments as stagnant seawater in combination with good notch toughness and tensile strength, said steel consisting essentially of from 16 to 30 percent chromium, from about 3 up to about 11 percent molybdenum, silicon present up to 1.5 percent, with the proviso that the "CMS" indicator represented by the sum of the chromium plus three times the amount of molybdenum plus three times the percentage of silicon is not less than 38 percent, nor above about 48 percent where good workability is desired, from 2 to about 8 percent nickel, up to less than 2 percent titanium, up to about 2 percent vanadium and up to about 2 percent columbium, with at least one element from the group consisting of titanium, vanadium and columbium being present in a small but effective amount to enhance the corrosion resistance in respect of steels produced by air melting and in which the "CMS" indicator is not above 41 percent, the sum total of titanium, vanadium and columbium not exceeding about 4 percent, up to 0.07 percent carbon, up to 2 percent aluminum, up to about 2 percent manganese, up to about 10 percent cobalt, up to about 4 percent tungsten, and the balance essen-

essentially iron.

2. A steel in accordance with claim 1 in which the "CMS" indicator is at least about 40 percent.

3. A steel in accordance with claim 2 in which the chromium content is from 22 to 28 percent.

4. A steel in accordance with claim 2 in which metal from the group consisting of titanium, vanadium and columbium is present in an amount of at least 0.15 percent.

5. A steel in accordance with claim 4 in which at least the element titanium is present.

6. A steel in accordance with claim 2 containing 18 to 22 percent chromium, about 5 to 10 percent molybdenum, up to about 1.5 percent silicon, a nickel content of about 2.5 to 6 percent, at least 0.2 percent of at least one metal from the group consisting of titanium, vanadium and columbium when the steels are produced by air melting, up to 0.5 percent aluminum, carbon present up to 0.06 percent and the balance essentially iron.

7. A steel in accordance with claim 6 in which the "CMS" indicator is at least 41 percent.

8. A steel in accordance with claim 2 containing from 22 to 28 percent chromium, about 3.5 to 8 percent molybdenum, up to about 1.5 percent silicon, a nickel content of about 2.5 to 6 percent, at least 0.2 percent of metal from the group consisting of titanium, vanadium and columbium when the steels are produced by air melting, up to 0.5 percent aluminum, carbon present up to 0.06 percent and the balance essentially iron.

9. A steel in accordance with claim 8 in which the

"CMS" indicator is at least 41 percent.

10. A steel in accordance with claim 1, which has been subjected to a final annealing treatment over a temperature range of about 1,900°F. to 2,200°F.

11. A stainless steel containing from 16 to 30 percent chromium, from about 0.5 up to about 11 percent molybdenum, up to 3 percent silicon, with the provisos that the "CMS" indicator represented by the sum of the chromium plus three times the amount of molybdenum plus three times the percentage of silicon is not less than 34 percent, nor above about 48 percent where good workability is desired, from 2 to about 8 percent nickel, up to less than 2 percent titanium, up to about 2 percent vanadium and up to about 2 percent columbium, with at least one element from the group consisting of titanium, vanadium and columbium being present in a small but effective amount to enhance the corrosion resistance in respect of steels produced by air melting and in which the "CMS" indicator is not above 38 percent, the sum total of titanium, vanadium and columbium not exceeding about 4 percent, carbon up to 0.1, up to 2 percent aluminum, up to about 2 percent manganese, up to about 10 percent cobalt, up to about 4 percent tungsten, and the balance essentially iron.

12. A steel in accordance with claim 2 in which carbon above about 0.06 percent is fixed.

13. A steel in accordance with claim 12 in which carbon above about 0.02 percent is fixed.

\* \* \* \* \*